

April 13, 1943.

C. MARSH

2,316,743

FLOTATION OF MOLYBDENITE

Filed Nov. 9, 1939

2 Sheets-Sheet 1

**FIG. 1.**



INVENTOR  
CORBIN MARSH,  
BY *Robert Ames Norton*  
ATTORNEY.

April 13, 1943.

C. MARSH

2,316,743

FLOTATION OF MOLYBDENITE

Filed Nov. 9, 1939

2 Sheets-Sheet 2

FIG. 2.



INVENTOR  
CORBIN MARSH,  
BY *Robert Ames Norton*  
ATTORNEY.

## UNITED STATES PATENT OFFICE

2,316,743

## FLOTATION OF MOLYBDENITE

Corbin Marsh, Old Greenwich, Conn., assignor to  
 American Cyanamid Company, New York,  
 N. Y., a corporation of Maine

Application November 9, 1939, Serial No. 303,589

5 Claims. (Cl. 209—166)

The present invention relates to improved methods and reagents for concentrating molybdenite by froth flotation.

In the past it has been considered very difficult to obtain molybdenite concentrates of sufficiently high grade by the use of heretofore known flotation agents and methods. In some instances the molybdenite containing ores also contain and are closely associated with a gangue material of the mica class from which it is very difficult to selectively float the molybdenite. In other cases the molybdenite may occur as relatively large masses of impure mineral containing quartz or pyrite in which case a high recovery of the molybdenite in a high grade concentrate requires grinding to a fineness far beyond the economical limits for such ores when employing previously known flotation agents.

In many ores molybdenite is found along with other mineral sulfides such as copper sulfide, iron sulfide, the various base metal sulfides or precious metal sulfides.

In the past two general procedures have been employed in the separation of molybdenite from the other metallic sulfides. Both of these procedures have depended on a flotation of the metal in the first instance. One of the processes employs a bulk float of both molybdenite and the other metallic sulfides and the separation is then effected by a suitable treatment of the concentrate obtained. The second procedure is a differential float, the molybdenite being depressed by the use of various reagents for example organic protective colloids such as starch in an alkaline solution. In both of these procedures the first flotation step is effected in the presence of promoters for ordinary metallic sulfides such as xanthates, dithiophosphates and the like.

According to the present invention, molybdenite is floated away from the other metallic sulfides, preferably by the use of an improved frothing agent which is not an efficient promoter for the new metallic sulfides. This frother is a mixture of higher aliphatic alcohols ranging from 6 to 10 carbon atoms admixed with hydrocarbons of the paraffin and terpene series. Improved grades and recoveries of molybdenite are obtained and when the molybdenite is present with other metallic sulfides, the recovery of these other sulfides by subsequent flotation procedure is advantageously affected.

The present invention is applicable to ores which contain molybdenite as the only or substantially the only valuable material and also to ores or concentrates in which molybdenite is admixed with other metallic sulfides, such as for example, copper sulfide. In the first case improved molybdenite recoveries are obtained in a single flotation procedure and the concentrate can be treated by cleaning or otherwise, to further increase the grade of molybdenite concen-

trate obtained. In the second instance the present invention adopts exactly the opposite course to that which was used in the past. Instead of carrying out a flotation procedure which results in a high recovery of the other metallic sulfides with or without molybdenite, a differential float is employed in which a first concentrate is obtained which shows a high recovery of molybdenite with a relatively low recovery of the other sulfides, followed if desired, by flotation procedures which will result in recovering a large proportion of the remaining sulfides. The first flotation operation is effected in the absence of ordinary sulfide promoters, producing a concentrate showing good recoveries of molybdenite. The tailings can then be treated by froth flotation in the presence of promoters for the sulfides.

Not all of the factors which influence the improved results of the present invention have been rigorously proved and I do not limit my invention to any particular theoretical proof. I believe, however, that at least one factor, and probably an important one in the case of ores containing both molybdenite and other sulfides, lies in the fact which I have discovered that ordinary sulfide promoters instead of increasing the recovery of molybdenite actually appear to lower this recovery. This extraordinary result which is contrary to the effect of ordinary sulfide promoters in ores containing sulfides, is one of the important factors in the improved results obtainable when the present invention is applied to ores containing molybdenite in admixture with other sulfides.

It is an advantage of the present invention that it is not particularly sensitive to pH changes over a considerable range. Excellent results can be obtained in the neutral circuits of many ores. In many other cases circuits of somewhat higher pH may be used. However, I have found that lime in large quantities is deleterious and much poorer recoveries are obtained if the ore pulp is conditioned with large quantities of lime. This action is apparently one which is due to the nature of the metal in the base used and not to its basicity as the addition of considerable amounts of bases of the alkali metals such as soda ash does not result in any serious lowering of the recovery. With some ores the addition of soda ash to produce a somewhat higher pH is actually helpful. Small amounts of lime, not exceeding in any case  $\frac{1}{2}$  lb. per ton of ore, do not appear to exert any serious deleterious action. However, if the amount of lime is increased materially beyond such amounts a rapid falling off in the recovery is noted. The relative insensitiveness of the process of the present invention to considerable changes in pH, provided large amounts of lime are not present, is one advantage of the present invention particularly when applied to ores containing sulfides other than molybdenite as a circuit pH can be chosen which will give the best separation between mo-

lybdenite and the other metallic sulfides without adversely affecting the total molybdenite recovered. The invention is therefore applicable to a wide range of molybdenite containing ores and does not require a critical pH control. The degree to which recoveries are adversely affected by the presence of lime varies widely with different ores but in every case lime in any considerable quantities is undesirable.

The invention will be described in greater detail in conjunction with the following specific examples and drawings in which:

Fig. 1 is a flow sheet representing steps in a procedure that may be used in carrying out a differential flotation of molybdenum and copper sulfides according to the present invention; and

Fig. 2 is a chart illustrating the effect that alkalies have on the recovery of molybdenite by flotation.

The flow sheet illustrated in Fig. 1 indicates steps that may be followed in carrying out the present invention. When the ore to be treated is a molybdenite ore substantially free from other sulfides or materials, a high recovery of  $MoS_2$  is obtained in a single step by subjecting the ore pulp to a froth flotation employing the improved frothing mixture composed of higher aliphatic alcohols, fuel oil and pine oil. When the ore also contains other mineral sulfides such as copper sulfide, a high grade  $MoS_2$  concentrate is first produced using the improved frother mixture and in the absence of promoters for the copper sulfide. If desirable, copper depressors can be added. The tailings are then subjected to a froth flotation in the presence of copper promoters to produce a second concentrate rich in copper. The first step may be carried out in a neutral circuit or in the case of some ores the pH may be increased by the use of certain alkalies or an alkali may be added in the second step along with the copper promoters. As pointed out heretofore, large quantities of lime depress molybdenite, therefore lime should not be used in large quantities to produce the  $MoS_2$  concentrate, but it can be used to a very good advantage in producing the subsequent copper concentrate. Figure 2 shows graphically the effect that soda ash and lime have on molybdenite flotation. The curves illustrate the fact that it is the alkalinity producing reagent used that affects the results rather than the actual alkalinity or pH changes.

#### EXAMPLE 1

A 600 gram sample of copper molybdenum ore from the Cananea Consolidated Copper Company, designated as No. 3-2 (República ore) was ground at 60% solids in a laboratory size steel rod mill and 0.5 lb. of lime per ton of ore was added to the grind. The ground pulp was trans-

ferred to a laboratory size Fagergren flotation machine and diluted to 22% solids with water. 0.09 lb. per ton of ore of a frother mixture containing 40% higher aliphatic alcohols, 40% fuel oil and 20% pine oil was mixed with the pulp and the pulp was then subjected to froth flotation. The rougher concentrate was returned to the flotation machine and cleaned by a re flotation. 0.1 lb. per ton of a copper promoter consisting of a 50-50 mixture of the sodium salts of diethyl dithiophosphoric acid and di-secondary butyl dithiophosphoric acid and 5.50 lbs. of lime per ton was used in the production of a second concentrate from the tailings. The results obtained in this test are shown in the following table:

Table 1

| Product         | Weight | Cu    | Assays<br>$MoS_2$ | Distribution |         |
|-----------------|--------|-------|-------------------|--------------|---------|
|                 |        |       |                   | Cu           | $MoS_2$ |
| Feed            | 100.00 | 1.87  | 0.076             | 100.00       | 100.00  |
| 1st concentrate | 1.51   | 26.26 | 4.270             | 21.21        | 96.33   |
| 1st clean tail  | 2.35   | 3.70  | 0.078             | 4.65         | 2.36    |
| 2nd concentrate | 7.32   | 16.29 | 0.002             | 63.67        | 0.13    |
| 2nd clean tail  | 1.39   | 2.14  | 0.001             | 1.60         | -----   |
| Tailing         | 87.43  | 0.19  | 0.001             | 8.87         | 1.18    |

The results of Example 1 recorded in Table 1 show that 96.33% of the  $MoS_2$  was obtained in the first flotation concentrate, associated with only 21.21% of the copper sulfide, which concentrate can very easily be improved in grade by the usual methods. This represents a marked improvement over prior methods in which promoters of sulfides are used to obtain a concentrate relatively high in both molybdenite and copper sulfide. It is also noted that the second concentrate represents a good copper recovery.

#### EXAMPLE 2

A series of flotation tests were conducted on a molybdenum ore using various frothers and frother mixtures as follows:

600 gram samples of 20 mesh molybdenum ore from the Molybdenum Corporation of America, containing about 4.14%  $MoS_2$  and a small amount of pyrite in a gangue composed principally of quartz, was ground at 60% solids in a laboratory size steel rod mill for a period of six minutes. The ground pulp was transferred to a laboratory size Fagergren flotation machine and diluted to 22% solids with water. Various frother reagents were added and conditioned with the pulp for a short time. Air was then admitted and the resulting froth was removed by skimming. The test products were filtered, dried, weighed and assayed. The metallurgical data resulting from the tests with the various frothing agents are shown in the following table:

Table 2

| Test No. | Feed<br>$MoS_2$ | Concentrate    |                  |       | Tailing          |       | Reagent                                                                                               | Lb./ton |
|----------|-----------------|----------------|------------------|-------|------------------|-------|-------------------------------------------------------------------------------------------------------|---------|
|          |                 | Weight<br>gms. | Assay<br>$MoS_2$ | Rec.  | Assay<br>$MoS_2$ | Dist. |                                                                                                       |         |
| 1        | Per cent        | Per cent       | Per cent         | (1)   | (1)              | ----- | Mixture of amyl alcohols. Boiling range 121-139° C.                                                   | 0.39    |
| 2        | -----           | (1)            | (1)              | (1)   | (1)              | ----- | Du Pont B23 alcohol. Boiling range 152-162° C.                                                        | 0.16    |
| 3        | -----           | (1)            | (1)              | (1)   | (1)              | ----- | Du Pont B25 alcohol. Boiling range 202-250° C. up.                                                    | 0.16    |
| 4        | 4.15            | 37.0           | 6.18             | 55.66 | 82.83            | 0.76  | Du Pont B27. Boiling range 133-202° C.                                                                | 0.16    |
| 5        | 4.14            | 33.5           | 5.57             | 58.89 | 79.25            | 0.91  | G. N. S. #8 pine oil.                                                                                 | 0.16    |
| 6        | 4.20            | 37.4           | 6.25             | 56.83 | 84.37            | 0.70  | (40% Du Pont alcohol B23; 30% #2 fuel oil; 20% G. N. S. #5 pine oil; 10% G. N. S. #8 pine tar oil)    | 0.16    |
| 7        | 4.21            | 37.0           | 6.25             | 57.55 | 85.52            | 0.65  | (40% Du Pont alcohol B23; 39.5% #2 fuel oil; 20% G. N. S. #5 pine oil; 0.5% G. N. S. #8 pine tar oil) | 0.16    |
| 8        | 4.09            | 39.4           | 6.57             | 54.72 | 87.90            | 0.53  | (40% Du Pont alcohol B27; 39.5% #2 fuel oil; 20% G. N. S. #5 pine oil; 0.5% G. N. S. #8 pine oil)     | 0.16    |

\* No assays. Results poor. \*G. N. S.—General Naval Stores.

An examination of Table 2 shows that the frothing reagents composed of a mixture of higher aliphatic alcohols having 6 to 10 carbon atoms, a paraffin hydrocarbon such as fuel oil, and a hydrocarbon of the terpene series such as pine oil, produced higher recoveries of molybdenite than were produced when such alcohols or hydrocarbons were used separately. Test #4 using a higher aliphatic alcohol resulted in a recovery of only 82.83% MoS<sub>2</sub> and test #5 using pine oil produced a concentrate containing only 79.2% MoS<sub>2</sub>, and yet mixtures of the two with fuel oil as shown in tests #6, 7, and 8 increased the MoS<sub>2</sub> recovery in the concentrate to 87.90%. This not only represents a very marked improvement in recovery but also an unexpected improvement.

What I claim is:

1. A process for the recovery of molybdenite by froth flotation which comprises subjecting an aqueous pulp containing molybdenite to a froth flotation operation in the presence of an effective amount of a collector for the molybdenite, said collector comprising a composition containing at least one higher aliphatic alcohol having six to ten carbon atoms, a hydrocarbon of the paraffin series and a hydrocarbon of the terpene series, the alcohol content of the composition being substantially 40%.

2. A process for the recovery of molybdenite by froth flotation which comprises subjecting an aqueous pulp containing molybdenite to a froth flotation operation in the presence of an effective amount of a collector for the molybdenite, said collector comprising a composition containing approximately 40% of a mixture of higher aliphatic alcohols having from six to ten carbon atoms, about 40% fuel oil and about 20% pine oil.

3. A process for the recovery of molybdenite by froth flotation which comprises subjecting an aqueous pulp containing molybdenite to a froth flotation operation in the presence of an effective amount of a collector for the molybdenite, said collector comprising a composition containing 40

5 approximately 40% of a mixture of higher aliphatic alcohols having from six to ten carbon atoms, about 40% fuel oil and about 20% pine oil, and in the absence of an effective amount of a collector for other sulfide ores.

4. A process for separating molybdenite from other metallic sulfides which comprises the steps of subjecting an ore containing both to froth flotation in the presence of an effective amount of a collector for the molybdenite which comprises a composition containing at least one higher aliphatic alcohol having six to ten carbon atoms, a hydrocarbon of the paraffin series and a hydrocarbon of the terpene series, and in the absence of an effective promoter for the other metallic sulfides, whereby a concentrate is obtained representing a high recovery of molybdenite in the ore and a relatively low recovery of the other metallic sulfides, subjecting the tailings to froth flotation in the presence of an effective amount of a promoter for said other sulfides producing a second concentrate representing a relatively high recovery of at least one of the other metallic sulfides, the alcohol content of the composition being substantially 40%.

5. A process for separating molybdenite from other metallic sulfides which comprises the steps of subjecting an ore containing both to froth flotation in the presence of an effective amount of a collector for the molybdenite which comprises a composition containing approximately 40% of a mixture of higher aliphatic alcohols having from six to ten carbon atoms, about 40% fuel oil and about 20% pine oil, and in the absence of an effective promoter for the other metallic sulfides, whereby a concentrate is obtained representing a high recovery of molybdenite in the ore and a relatively low recovery of the other metallic sulfides, subjecting the tailings to froth flotation in the presence of an effective amount of a promoter for said other sulfides producing a second concentrate representing a relatively high recovery of at least one of the other metallic sulfides.

CORBIN MARSH.